# EUROPEAN PATENT SPECIFICATION

(11) **EP 1 537 260 B1**
(45) Date of publication and mention of the grant of the patent: **04.11.2009**
(21) Application number: 03754576.1
(22) Date of filing: 15.09.2003
(51) Int. Cl.: D01F 1/09, D01F 6/60, D01F 8/12, D04H 3/12

(54) **METHOD OF REDUCING STATIC IN A SPUNBOND PROCESS**
VERFAHREN ZUR REDUZIERUNG VON STATISCHEN LADUNGEN IN EINEM SPUNBONDVERFAHREN
PROCEDE DE REDUCTION DE L'EFFET STATIQUE DANS UN PROCESSUS FILE-LIE

(30) Priority: 13.09.2002 US 410557 P
(43) Date of publication of application: 08.06.2005
(73) Proprietor: Cerex Advanced Fabrics, Inc., Cantonment, FL 32533 (US)
(72) Inventor: ORTEGA, Albert, E., Pensacola, FL 32514 (US)
(74) Representative: Perry, Robert Edward
(86) International application number: PCT/US2003/028909
(87) International publication number: WO 2004/025004

(56) References cited:
- EP-A- 0 331 876
- US-A- 5 116 897
- US-A- 5 145 727
- US-A- 5 237 009
- US-A- 5 814 688

## Description

### Field of Invention

This invention relates to a method of reducing static in a spunbonded process. The addition of an antistatic agent or agents in the melt allows static to be dissipated providing an advantageous spunbond process.

### Background of Invention

Most textile processes generate some amount of static due to friction. Static is generated in spinning processes by air passing across filaments and by filaments rubbing over other surfaces. In the production of yarn, this static is commonly dissipated by the addition of finish to the filaments in a filament bundle or threadline. Finishes typically contain lubricating oils, water, antistatic agents and other additives to impart special properties to the fiber or to enhance the ability to process the fiber.

However, in the production of spunbonded fabrics, finish is usually not applied to the filaments. Spunbond processes typically use one or more extruders to melt polymer resins. The melt stream is then filtered and pumped to a spinneret forming filaments that are typically quenched with cool air. Bicomponent or multicomponent spinning methods as described in U.S. patent numbers 3,968,307; 4,052,146; 4,406,850; 4,424,257; 4,424,258; 4,830,904; 5,534,339; 5,783,503; 5,895,710; 6,074,590 and 6,207,276, can also be used to make multiconstituent filaments with various properties. In a bicomponent or multicomponent spinning system, the antistatic additive should at least be added to one of the components that will be on the surface of the filaments.

The filaments are attenuated and drawn pneumatically through a jet or slot device and deposited onto a collection surface to form a web. Air is commonly used as the attenuation medium. A vacuum can also be used to move the air through the attenuation device. Static is generated by air rubbing over the filaments in the slot or jet device. Some level of defects and efficiency loss is caused by static. Static can be reduced somewhat but not eliminated by increasing the moisture in the environment surrounding the filaments. Reducing or eliminating the static would be beneficial.

The web is then bonded together to produce a strong, coherent fabric. Filament bonding is typically accomplished either thermally or chemically, i.e., autogenously. Thermal bonding is accomplished by compression of the web of filaments between the nips of a pair of cooperating heating calender rolls. In autogenous bonding of nylon filaments, the web of filaments is transported to a chemical bonding station or "gashouse" which exposes the filaments to an activating agent (i.e., HCl) and water vapor. Water vapor enhances the penetration of the HCl into the filaments and causes them to become tacky and thus amenable to bonding. The web may also be bonded using adhesives to "glue" fibers together to render the fibers cohesive. Upon leaving the bonding station, the web passes between rolls, which compress and bond the web. Even distribution of mass is necessary to provide minimal variation in fabric physical properties and to impart uniformly, good strength properties to the fabric.

High levels of static cause processing problems in both drawing systems listed above. In the jet process, high static levels cause individual filaments or group of filaments to cling to the nearest conductive surface. This creates a small semi circle defect in the fabric. In the slot process, high levels of static have a similar effect. Individual filaments cling to conductive surfaces and interrupt the normal mass flow creating a fabric defect. In both attenuation systems, static affects the formation of the web reducing the uniformity of the fabric appearance. EP0331876 discloses polyamide shaped articles and their manufacture. Additives that can be employed include antistatic agents.

A process that has little to no static will consistently provide a more uniform fabric at higher efficiencies which is extremely beneficial.

### Brief Summary

The subject invention provides a process according to claim 1. In the process, an antistatic agent or agents is added in the polymer melt enabling the efficient production of single or multicomponent spunbond fabric with acceptable uniformity. In an embodiment specifically exemplified herein, the spunbonded process uses nylon resin and attenuates filaments with a slot device. In a preferred embodiment, a reduction in static is observed by the addition of about 0.25% of an antistatic additive on the sheath side. In another preferred embodiment, an improved process with very low static is provided by the addition of about 0.75% antistatic additive on the sheath side of nylon filaments in a slot attenuation process.

The addition of antistatic agents benefits various spinning processes including but not limited to single, bicomponent, and multicomponent polymer systems. In bicomponent or multicomponent systems, the antistatic additive should at least be added to one of the components that will be on the surface of the filaments. A slot or jet attenuation device can be used in any of these spin systems to draw the filaments to the desired denier and deposit them onto a surface to form a web. The web can be bonded thermally, ultrasonically or chemically, i.e., autogenously.

### Detailed Disclosure

In the following detailed description of the subject invention and its preferred embodiments, specific terms are used in describing the invention; however, these are used in a descriptive sense only and not for the purpose of limitation.

High levels of static cause filaments to hang on any conductive surface until the static on the surface of that filament is dissipated. This interrupts the mass flow creating a fabric defect. Extremely high levels of static cause the filaments to cling to the outlet end of the jet tube creating a section of web with lower mass and a section with higher mass once the static is dissipated and the filaments are released from the tube. In the slot process, high levels of static have a similar effect; individual filaments cling to conductive surfaces and interrupt the normal mass flow creating a fabric defect. Extremely high levels of static frequently interrupt the normal mass flow creating large fabric defects. In both attenuation systems static affects the formation of the web reducing the uniformity of the fabric.

This invention concerns the addition of antistatic agents to spunbond processes to reduce fabric defects and to improve fabric uniformity. In one embodiment, an antistatic additive or a combination of antistatic additives, such as PTSS 1378, available from PolyTech South, Inc. and comprising polycaprolactam (nylon 6), sulfonic acids, C₁₀-C₁₈ alkane and sodium salts is added through an auger into the throat of one extruder used to make nylon 6,6 filaments.

Other antistatic additives including, but not limited to, those described in U.S. Patent Nos. 6,369,159; 6,150,446; 6,123,990; 5112528; 5,744,573; 5,023,036; 5,237,009; 5,342,889; 5,084,504; 5,179,155; 5,659,058; 5,116,897; and 5,025,922 can also be used.

Various nylon polymers including, but not limited to, nylon 6; nylon 6,6; nylon 6,10; nylon 6,12; nylon 11; nylon 12; nylon copolymers, and mixtures thereof can be utilized in the process of the present invention.

Antistatic materials that can be used according to the subject invention include, but are not limited to, saccharine; quarternary ammonium salts; homo- and co-polymers of epihalohydrin; N,N,-Bis(hydroxyethyl) alkylamine; chain extended polyoxiranes; aromatic sulfanomides and similar antistatic agents.

In one embodiment, the antistatic agent can be ethylene oxide and at least one heterocyclic co-monomer. In this embodiment, the co-monomer can be in the range of from about 5% to about 95% by weight, wherein the cyclic co-monomer comprises a ring comprising an oxygen atom and at least two carbon atoms. Such compounds include, for example, epihalohydrin or propylene oxide.

Also, the antistatic agent can be a polar antistatic agent comprising a mixture of at least one polar organic compound having at least 5 carbon atoms and a compound having at least 3 heteroatoms. The compounds used in this mixture can be, for example, polyethers, crown ethers, polyols, polyimines, polyamines, polymers derived from pyridine, macrocyclic aza compounds, polysulfides and polyphosphines, and salts of protic acids that are solvated or complexed in a polar organic compound. The salt may be, for example, LiClO₄, LiCF₃SO₃, NaClO₄, LiBF₆, NaBF₆, KBF₆, NaCF₃SO₃, KClO₄, KPF₆, KCF₃SO₃, Ca(ClO₄)₂, Ca(PF₆)₂, Ca(CF₃SO₃)₂, Mg(ClO₄)₂, Mg(CF₃SO₃)₂, Zn(ClO₄)₂, Zn(PF₆)₂ or Ca(CF₃SO₃)₂.

In additional embodiments, the antistatic agent can be styrene polymers; the copolymerization product of ethylene oxide with a heterocyclic monomer or vinyl type monomer; low molecular weight polyether oligomers; carbon particles; trineoalkoxy amino zirconate; trineoalkoxy sulfonyl zirconate; or a compound of the general formula wherein R is a C₁₋₉ alkyl group or hydrogen, Z is a difunctional chain modifier group, R' is a C₁₋₄ alkyl group or hydrogen and x and y are between about 10 and about 50. In a specific embodiment, the compound can have the formula where R is a C₁₋₅ alkyl group or hydrogen, Z is a difunctional chain modifier group, R' is a C₁₋₄ alkyl group or hydrogen and x and y are each between about 20 and about 40.

In the embodiment depicted by the formulae shown above, the antistatic agent is a linear polyester preferably prepared via the base-catalyzed transesterification of dimethyl azelate with a N-methyldiethanol amine-initiated ethylene oxide/propylene oxide block polymer. The optimum length of propylene oxide and ethylene oxide chains in general has been optimized and the optimum length is known from the literature. The regulation of the chain to the desired length is easily accomplished by one ordinarily skilled in the art by adding proper molar equivalents in a stepwise manner. Chain modifiers are known to those skilled in the art. By way of illustration, the preferred chain modifiers are difunctional. The useful difunctional chain modifiers preferably have acidic or nearly analogously reactive functionality. Preferred chain modifiers are dibasic acids having less than 18 carbon atoms and derivatives thereof Exemplary modifiers are azelaic acid and alkylazelates. The oxyalkylene chains are preferably end-capped. See, U.S. Patent No. 5,116,897.

The filaments can be drawn and attenuated, either by a slot or jet device and deposited onto a surface forming a web. The web is then ultrasonically, thermally or chemically bonded. In a specific embodiment, thermal bonding is accomplished by compression of the web of filaments between the nips of a pair of cooperating heating calender rolls set at around 220 ° C for nylon filaments.

In autogenous bonding of nylon filaments, the web of filaments is transported to a chemical bonding station or "gashouse" that exposes the filaments to an activating agent (i.e., HCl) and water vapor. Water vapor enhances the penetration of the HCl into the filaments and causes them to become tacky and thus amenable to bonding. The web may also be bonded using adhesives to "glue" fibers together to render the fibers cohesive. Upon leaving the bonding station, the web passes between rolls, which compress and bonds the web.

In a specific embodiment, a reduction in static of about 44% is achieved with the addition of 0.25% of PTSS 1378, available from PolyTech South, Inc. Thus, an antistatic agent comprising polycaprolactum (nylon 6), sulfonic acids, C10-C18 alkane and sodium salts, can be added to the extruder feeding the sheath side of a bicomponent filament spinning system with a slot attenuation system. The same polymer can be fed to an extruder feeding the core side and to an extruder feeding the sheath side of a pilot line capable of bicomponent filament spinning. Higher addition levels give lower static levels up to the point where the majority of the static has been dissipated.

If a single component spinning system with a single extruder is used for this embodiment, it is preferable to add at least 0.25% to the entire melt stream. Levels as low as 0.1 % can reduce static; however, the reduction may not be sufficient. Thus, the invention contemplates the addition of at least about 0.2% of the antistatic agent.

The filaments can then be drawn by a slot or jet attenuation device and deposited onto a surface forming a web. The web can then be calendered at 215° C engraved roll temperature and 205° C smooth roll temperature.

For a bicomponent or multicomponent spinning process, the addition of an antistatic agent or agents is required only for the portion of the filaments that will be on the surface of the filaments. Adding the antistatic agent or agents to the internal section of a multicomponent filament is not as effective as adding it to the surface of the filament.

Any man-made polymer can be used, such as, but not limited to, polycaprolactum, polyamide, polyester, polyethylene, polypropylene, polylactic acid, poly(trimethylene terephthalate), polyvinyl alcohol, vinyl acetate, nylon 6, nylon 6,6, nylon 10, nylon 11 and nylon 12. Blends and copolymers of man-made polymers can also be used. Also, mixtures, blends or copolymers can be used as taught in U.S. Patents 5,431,986 and 5,913,993. In one embodiment, polyethylene, polypropylene, and/or polyester can be added to the nylon material. This produces a softer feel and increases water repellency. In the case of polyethylene, the polyethylene should have a melt index between about 5 grams/10 min and about 200 grams/10 min and a density between about 0.85 grams/cc and about 1.1 grams/cc. The polyethylene can be added at a concentration of about 0.05% to about 20%.

Nylon filaments produced according to the process of the subject invention may be bonded chemically, ultrasonically, or thermally. In one embodiment, HCl gas and water vapor can be applied to achieve bonding as described in U.S. Patent 3,853,659. In another embodiment, the filaments may be heated to, for example, between 180° C and about 250° C. Preferably, the filaments are heated to between about 200° C and 235° C.

Thus, in a preferred embodiment, the subject invention provides a method of producing a spunbonded nonwoven fabric comprising the steps of forming a melt blend, either in a master batch or a base resin, of polymer and one or more antistatic agents, extruding the blend in the form of a plurality of continuous filaments, directing the filaments through an attenuation device and drawing the filaments, depositing the filaments onto a collection surface to form a web and bonding the filaments of the web. The filaments can be made from, for example, nylon, polyester, acrylic, polyethylene, polypropylene, polybutylene terephtalate, poly(trimethylene terephthalate), polylactic acid polymers or a combination of these polymers.

A further embodiment provides a method of producing a spunbonded nonwoven fabric comprising the steps of forming two or more melt blends, either in a master batch or a base resin, of polymer and one or more antistatic agents, extruding the blends through separate extruders into the form of a plurality of continuous multicomponent filaments, directing the filaments through an attenuation device and drawing the filaments, depositing the filaments onto a collection surface to form a web and bonding the filaments of the web.

The components of the filaments can be made from, for example, nylon, polyester, acrylic, polyethylene, polypropylene, poly(trimethylene terephthalate), polylactic acid polymers, polybutylene terephthalate, ethylene vinyl alcohol, polyvinyl alcohol, vinyl acetate or a combination of these polymers.

A further embodiment provides a method of producing a spunbonded nonwoven fabric comprising the steps of forming one or more melt blends, either in a master batch or a base resin, of polymer and one or more antistatic agents, extruding the blend or blends through separate extruders into the form of a plurality of continuous multicomponent filaments with the blend or blends of polymer and one or more antistatic agents forming a portion of the surface of the filaments, directing the filaments through an attenuation device and drawing the filaments, depositing the filaments onto a collection surface to form a web and bonding the filaments of the web. The components of the filaments can be made from, for example, nylon, polyester, acrylic, polybutylene terephthalate, polyethylene, polypropylene, ethylene vinyl alcohol, polyvinyl alcohol, vinyl acetate, poly(trimethylene terephthalate), polylactic acid polymers or a combination of these polymers; and the attenuation device can be, for example, a slot device or a jet.

For single component, bicomponent and multicomponent slot attenuation spunbound process, the static level as measured one half inch or less below the outlet of the attenuation device is between -2 kilovolt per inch to 2 kilovolt per inch. Preferably, at least 5% of the total surface area of all the filaments and each of the filaments produced according to the present invention is a slot device are nylon polymer.

Advantageously, the fabric produced according to the process of the present invention has lower static resistivity and faster static dissipation rates or decay than a fabric produced without antistatic additives.

Following are examples which illustrate procedures for practicing the invention. These examples should not be construed as limiting. All percentages are by weight and all solvent mixture proportions are by volume unless otherwise noted.

### Example 1

An antistatic additive, PTSS 1378, available from PolyTech South, Inc. and comprising polycaprolactam (nylon 6), sulfonic acids, C₁₀-C₁₈ alkane and sodium salts was added at various levels to a slot pilot line running nylon 6,6 polymer.

The slot pilot line has bicomponent spinning capability. The line was set up to run the same polymer through two extruders and through two polymer delivery manifolds in a sheath - core system. The antistatic additive was added only to the sheath side. This is not a requirement but was done to conserve the amount of antistatic additive since there was a limited supply. Static was initially measured where the filaments exit the slot attenuation device with no antistatic additive present.

The PTSS 1378 antistatic additive was added at 0.25, 0.5, 0.75 and 1 percent and static was measured where the filaments exit the slot attenuation device. Since static charge only resides on the outside of the filament there was no need to supply the antistatic additive to the core side of the filaments. The additive was only added to the sheath side of the bicomponent spinning system. The antistatic additive could be added at the percentages listed in Table 1 to the entire polymer flow stream if only one extruder was used. Static was measured with a hand held static meter, model 212, manufactured by Electro-Tech Systems, Inc. Table 1 lists the results for the different levels of antistatic additive.

**Table 1.**

| Static measurements for different levels of antistatic additive | |
|---|---|
| Level of PTSS 1378 (%) | Static where filaments exit the slot attenuation device (Kilovolts/inch) |
| 0 | 4-7 |
| 0.25 | 2-2.5 |
| 0.50 | 1-1.5 |
| 0.75 | 0.6-1.6 |
| 1.0 | 0.6-1.6 |

The results show a decrease in static up to the addition of 0.75% PTSS 1378 antistatic additive to the sheath side of the filaments. Lowering the static to the level observed provided desirable spinning performance and allowed the production of fabric with acceptable uniformity.

Other antistatic additives can be used as previously referenced. Other polymer resins, copolymer resins, blends of resins or mixtures of resins can also be used.

### Example 2

An antistatic additive such as that described in Example 1 can be added to a spunbond process using jet attenuators and running nylon 6,6 polymer or a blend of nylon 6,6 and nylon 6 as described in U.S. Patent 5,431,986. The more rapid dissipation of static in these processes can be used to advantageously reduce defects and improve fabric uniformity.

### Example 3

An antistatic additive can be added to the sheath side of a bicomponent spinning process to reduce static as described in Example 1. The core side of the filament can contain any other polymer that can be processed in a bicomponent or multicomponent spinning system to produce acceptable filaments. The attenuation device can be either a slot system as described in Example 1 or a jet system as described in Example 2. The more rapid dissipation of static from the sheath portion of the filament in these processes improves efficiency, reduces defects and improves fabric uniformity.

### Example 4

An antistatic additive can be added to the surface of a multicomponent filament spunbond process similar to the system described in Example 1. The core side of the filament can contain any other polymer that can be processed in a multicomponent spinning system to produce acceptable filaments. The attenuation device can be either a slot system as described in Example 1 or a jet system as described in Example 2. The more rapid dissipation of static from the surface portion of the filament in these processes improves efficiency, reduces defects and improves fabric uniformity.

### Example 5

The resin with antistatic materials described in Example 1 was added to the slot draw pilot line described in Example 1. These materials were compounded in nylon 6. A master batch of nylon 6, optical brightener and TiO₂ was also mixed with the compounded resin with the antistatic additives and added to the extruder using an auger. Approximately, 1.3% of the master batch resin and 1% of the antistatic resin was added to the sheath side of the bicomponent slot draw pilot line. Humidifiers were turned on in the spinning operations area to increase the humidity.

Static was measured using the hand held static meter, model 212, manufactured by Electro-Tech Systems, Inc. at 0.05 to 0.09 kilovolts per inch. This trial was repeated a second time and static was measured at 0.8 to 1.3 kilovolts per inch. The trial was replicated a third time and the static was measured at 0.5 to 1.7 kilovolts per inch.

Fabric samples were produced at various basis weights. These samples should have lower static resistivity, and faster static dissipation rates or static decay than samples made with no antistatic additives. These samples should also have lower static resistivity and faster static dissipation rates or static decay than commercially existing nylon spunbonded fabrics without antistatic additives.

### Example 6

An antistatic additive was added to the slot draw pilot line described in Example 1. This material was compounded in nylon 6,6. The resin is commercially available and it included a sulfonated compound and a phosphorous compound similar to that described in U.S. patent 5,045,580. A master batch of nylon 6, optical brightener and TiO₂ was also mixed with the commercial resin with the antistatic material and added to the extruder using an auger. The master batch was supplied by Clariant. The mixture was added to the sheath side of the bicomponent slot draw pilot line described in Example 1. This mixture was added at various levels shown in Table 2. The mixture can also be added at the levels shown in Table 2 to the entire polymer stream if only one extruder was used.

Table 2 lists the static measurement results for different levels of antistatic resin. Fabric samples were made at the levels listed in the table.

**Table 2.**

| Static measurements for different levels of an antistatic additive | | |
|---|---|---|
| Level of Resin with antistatic additive (%) | Level Clariant AF 03732001 (%) | Static where filaments exit the slot attenuation device (Kilovolts/inch) |
| 1* | 1.3 | 4.5 - 7.0 |
| 2 | 1.3 | 1.88 - 2.6 |
| 3 | 1.3 | 0.38 - 0.53 |
| 3.17 | 1.13 | 0.5 |
| 4 | 1.3 | 0.32-0.44 |
| 4.51 | 0.79 | 0.31 - 0.42 |
| 5.18 | 1.12 | 0.19 - 0.26 |
| 6 | 1.3 | 0.17 - 0.20 |

| | | |
|---|---|---|
| * Comparative example | | |

The results show a substantial decrease in static up to the addition of about 3% of the resin with the antistatic material. Lowering the static to the level observed provided acceptable spinning performance and allowed the production of fabric with desirable uniformity. These fabric samples should have lower static resistivity and faster static dissipation rates or static decay than samples made with no antistatic additives. These samples should also have lower static resistivity and faster static dissipation rates or static decay than commercially existing nylon spunbonded fabrics without antistatic additives.

Other antistatic additives compounded in nylon 6 or nylon 6,6 can also be used as described in previous referenced patents and in U.S. patents 5,814,688 and 5,955,517. It is not a requirement of the invention to use master batches of the antistatic additive. Antistatic additives can be included in the base resin providing the resin supplier has the capability to incorporate these antistatic additives in the polymerization process.

### Example 7

Two other resins with antistatic additives were added to the sheath side of the slot draw pilot line described in Example 1. These materials were compounded in nylon 6,6. These materials can be added to the entire polymer stream if only one extruder was used. It is not a requirement of the invention to use master batches of the antistatic additives. Antistatic additives can be included in the base resin providing the resin supplier has the capability to incorporate these antistatic additives in the polymerization process. Table 3 lists the static measurement results for different levels of antistatic resins.

**Table 3.**

| Static measurements for different levels of a third and fourth antistatic additive | | |
|---|---|---|
| Resin with antistatic additive (%) | Level of Resin with antistatic additive (%) | Static where filaments exit the slot attenuation device (Kilovolts/inch) |
| None | 0 | 2 - 14 |
| 3A46 | 2 | 1.5 - 4.0 |
| 3A46 | 4 | 0.8 - 1.3 |
| 3A46 | 6 | 0.2 - 1.0 |
| 422 | 3 | (-0.47) - (-0.38) |

The results show a substantial decrease in static up to the addition of about 6% of the 3A46 resin with the antistatic materials. The results also show a low static level for the addition of 3% of resin 422.

## Claims

1. A method of producing a spun-bonded non-woven fabric, comprising the steps of: forming a melt blend of at least one polymer and at least one antistatic agent, extruding said blend in the form of a plurality of filaments, directing the filaments through an attenuation device and drawing the filaments to orient them, depositing the filaments onto a collection surface to form a web, and bonding the filaments of the web; wherein the fabric has lower static resistivity and faster static dissipation rate or delay than a fabric produced without the antistatic agent, and wherein the static level, measured at about one half inch (12.7 mm) below the outlet of the slot attenuation device, is between -2 and 2 kilovolt per inch (-102 and 102 kV/mm).

2. A method according to claim 1, wherein the filaments comprise nylon, polyester, an acrylic polymer, polyethylene, polypropylene, polybutylene terephthalate, poly(trimethylene terephthalate) or a polylactic acid, or a combination of these polymers.

3. A method according to claim 2, wherein the filaments comprise nylon 6; nylon 6,6; nylon 6,10; nylon 6,12; nylon 11; nylon 12; or a nylon copolymer; or a combination of these nylon polymers.

4. A method according to claim 1, which utilises two or more melt blends of polymer.

5. A method according to claim 1, wherein the attenuation device is a slot device.

6. A method according to claim 1, wherein the attenuation device is a jet.

7. A method according to claim 1, wherein the antistatic agent is selected from saccharine; quaternary ammonium salts; homo- and co-polymers of epihalohydrin; N,N-bis(hydroxyethyl)alkylamines; chain-extended polyoxiranes; aromatic sulfonamides; styrene polymers; copolymerization products of ethylene oxide with a heterocyclic monomer or vinyl-type monomer; low molecular weight polyether oligomers; carbon particles; trineoalkoxy amino zirconates; trineoalkoxy sulfonyl zirconates; and compounds of the formula R-CH₂-N[CH₂CH₂O(C₂H₄O)_{y}(C₃H₆O)ₓZR']₂ wherein R is H or C₁₋₉ alkyl, Z is a difunctional chain modifier group, R' is H or C₁₋₄ alkyl, and x and y are between 10 and 50.

8. A method according to claim 7, wherein R is H or C₁₋₉ alkyl, R' is H or C₁₋₄ alkyl, and x and y are between 20 and 40.

9. A method according to claim 1, wherein the antistatic agent comprises a polymer of ethylene oxide and at least one heterocyclic co-monomer.

10. A method according to claim 1, wherein the antistatic agent comprises a mixture of at least one polar organic compound having at least 5 carbon atoms and a compound having at least 3 heteroatoms.

11. A method according to claim 1, wherein the antistatic agent comprises a sulfonic acid, a C₁₀-C₁₆ alkane, and sodium salts.

12. A method according to any preceding claim, wherein the antistatic agent comprises one or more of polyethers, crown ethers, polyols, polyimines, polyamines, polymers derived from pyridine, macrocyclic aza compounds, polysulfides and polyphosphines, and salts of protic acids that are solvated or complexed in a polar organic compound.

13. A method according to any preceding claim, wherein said static level is between -1 and 1 kilovolt per inch (-51 and 51 kV/mm).

14. A method according to any preceding claim, wherein at least about 5% of the surface area of each filament is made of a nylon polymer.

15. A method according to any preceding claim, wherein at least about 5% of the total surface area of all filaments is made of a nylon polymer.

16. A method according to any preceding claim, comprising the steps of: forming one or more melt blends of polymer and one or more antistatic agents either in a master batch or a base resin, extruding said blend or blends through separate extruders into the form of a plurality of multicomponent filaments with the blend or blends of polymer and one or more antistatic agents forming a portion of the surface of the filaments, directing the filaments through an attenuation device, drawing the filaments to orient them, depositing the filaments onto a collection surface to form a web, and bonding the filaments of the web.

17. A method according to any preceding claim, wherein the fabric is uniform.

## Patentansprüche

1. Verfahren zur Herstellung eines im Spunbondverfahren hergestellten nichtgewebten Stoffes, umfassend die Schritte: Ausbilden einer Schmelzmischung von mindestens einem Polymer und mindestens einem antistatischen Agens, Extrudieren der besagten Mischung in Gestalt einer Vielzahl von Filamenten, Ausrichten der Filamente durch eine Verdünnungseinrichtung, und Ziehen der Filamente, um sie zu orientieren, Absetzen der Filamente auf einer Sammleroberfläche, um ein Gewebe zu bilden, und Bonden der Filamente des Gewebes, wobei der Stoff einen geringeren statischen spezifischen Widerstand hat und eine schnellere statische Entladungsrate oder -verzögerung als ein Stoff, der ohne das antistatische Agens hergestellt ist, und wobei das statische Niveau, gemessen ungefähr ein halbes Zoll (12.7 mm) unterhalb des Ausgangs der Schlitz-Verdünnungseinrichtung, zwischen -2 und 2 Kilovolt je Zoll (-102 und 102 vK/mm) beträgt.

2. Verfahren gemäss Anspruch 1, bei dem die Filamente Nylon, Polyester, ein Acrylpolymer, Polyethylen, Polypropylen, Polybutylen, Terephthalat, Poly(trimethylen-terephthalat) oder eine polylaktische Säure oder eine Kombination dieser Polymere ist.

3. Verfahren gemäss Anspruch 2, bei dem die Filamente Nylon 6; Nylon 6,6; Nylon 6,10; Nylon 6,12; Nylon 11; Nylon 12 oder ein Nylon-Copolymer umfassen oder eine Kombination dieser Nylonpolymere.

4. Verfahren gemäss Anspruch 1, welches zwei oder mehr Schmelzmischungen vom Polymer einsetzt.

5. Verfahren gemäss Anspruch 1, bei dem die Verdünnungseinrichtung eine Schlitzeinrichtung ist.

6. Verfahren gemäss Anspruch 1, bei dem die Verdünnungseinrichtung eine Düse ist.

7. Verfahren gemäss Anspruch 1, bei dem das antistatische Agens ausgewählt ist aus Saccharin, quaternäre Ammoniumsalze, Homo- und Co-Polymere von Epihalohydrin, N,N-bis (Hydroxyäthyl) Alkylamine; kettenverlängerte Polyoxirane; aromatische Sulfonamide; Styrol-Polymere; Copolymerisationsprodukte von Ethylenoxid mit einem heterozyklischen Monomer oder einem Monomer des Vinyltyps, niedrig molekular gewichtige Polyätheroligomere; Kohlenstoffpartikel; Trineoalkoxy-Aminozirkonate; Trineoalkoxy-Sulfonylzirkonate; und Verbindungen der Formel R-CH₂-N[CH₂CH₂O(C₂H₄O)y(C₃H₆O)ₓZR']₂, wobei R H oder C₁₋₉ Alkyl ist, Z eine difunktionale Kettenmodifizierungsgruppe ist, R' H oder C₁₋₄ Alkyl ist, und x und y zwischen 10 und 50 liegen.

8. Verfahren gemäss Anspruch 7, bei dem R H oder C₁₋₉ Alkyl ist, R' H oder C₁₋₄ Alkyl ist und x und y zwischen 20 und 40 sind.

9. Verfahren gemäss Anspruch 1, bei dem das antistatische Agens ein Polymer von Ethylenoxid und mindestens einem heterozyklischen Co-Monomer umfasst.

10. Verfahren gemäss Anspruch 1, bei dem das antistatische Agens eine Mischung von mindestens einer polaren organischen Verbindung mit mindestens 5 Kohlenstoffatom und einer Verbindung mit mindestens 3 Heteroatomen umfasst.

11. Verfahren gemäss Anspruch 1, bei dem das antistatische Agens eine Sulfonsäure, ein C₁₀-C-₁₆ Alkan und Natriumsalze umfasst.

12. Verfahren gemäss einem der vorstehenden Ansprüche, bei dem das antistatische Agens einen oder mehrere Polyäther, Kronenäther, Polyole, Polyimine, Polyamine, Polymere, die von Pyridin abgeleitet sind, makrozyklische Azoverbindungen, Polysulfide und Polyphosphine, und Salze von protischen Säuren umfasst, die in einer polaren organischen Verbindung solvatisiert oder komplexiert sind.

13. Verfahren gemäss einem der vorstehenden Ansprüche, bei dem das besagte statische Niveau zwischen -1 und 1 Kilovolt je Zoll (-51 und 51 kV/mm) ist.

14. Verfahren gemäss einem der vorstehenden Ansprüche, bei dem mindestens 5% des Oberflächenbereichs von jedem Filament aus einem Nylonpolymer besteht.

15. Verfahren gemäss einem der vorstehenden Ansprüche, bei dem mindestens 5% des gesamten Oberflächenbereichs von allen Filamenten aus einem Nylonpolymer besteht.

16. Verfahren gemäss einem der vorstehenden Ansprüche, umfassend die Schritte: Ausbilden einer oder mehrerer Schmelzmischungen von einem Polymer und einem oder mehreren antistatischen Agenzien, entweder in einem Hauptlos oder einem Basisharz, Extrudieren der besagten Mischung oder Mischungen durch getrennte Extruder in die Gestalt einer Vielzahl von vielfachzusammengesetzten Filamenten, wobei die Mischung oder Mischungen von Polymer und einem oder mehreren antistatischen Agentien einen Anteil der Oberfläche der Filamente ausbilden, Ausrichten der Filamente durch eine Verdünnungseinrichtung, Ziehen der Filamente, um sie zu orientieren, Absetzen der Filamente auf einer Sammleroberfläche, um ein Gewebe zu bilden, und Bonden der Filamente an das Gewebe.

17. Verfahren gemäss einem der vorstehenden Ansprüche, bei dem der Stoff gleichförmig ist.

## Revendications

1. Procédé pour la fabrication d'un non-tissé de type spunbond, comprenant les étapes: former un mélange fondu d'au moins un polymère et au moins un agent antistatique, extruder ledit mélange en forme d'une pluralité de filaments, diriger les filaments à travers un dispositif d'atténuation et tirer les filaments pour les orienter, déposer les filaments sur une surface de collection pour former un tissu, et relier les filaments du tissu, où l'étoffe présente une résistance spécifique statique plus petite et un ralentissement ou taux de déchargement statique plus élevé qu'une étoffe qui a été fabriquée sans ledit agent antistatique, et où le niveau statique, mesuré environ un-demi pouce (12.7 mm) en dessous de la sortie du dispositif d'atténuation à fente, est entre -2 et 2 kilovolt par pouce (-102 et 102 vK/mm).

2. Procédé selon la revendication 1, où les filaments comprennent du nylon, du polyester, un polymère acrylique, un polyéthylène, un polypropylène, un poly butylène, du téréphtalate, du poly (tri méthylène-téréphtalate) ou un acide poly lactique ou une combinaison de ces polymères.

3. Procédé selon la revendication 2, où les filaments comprennent du nylon 6; du nylon 6,6; du nylon 6,10; du nylon 6,12; du nylon 11; du nylon 12 ou un copolymère de nylon ou une combinaison de ces polymère de nylon.

4. Procédé selon la revendication 1, lequel utilise deux ou plus de mélanges fondus d'un polymère.

5. Procédé selon la revendication 1, où le dispositif d'atténuation est un dispositif à fente.

6. Procédé selon la revendication 1, où le dispositif d'atténuation est une buse.

7. Procédé selon la revendication 1, où l'agent antistatique est choisi parmi de la saccharine, des sels d'ammonium quaternaires, des homopolymères et des copolymères de l'epihalohydrine, des N,N-bis (hydroxyéthyle) alkyle amines; des polyoxiranes à chaine prolongée; des sulfamidés aromatiques; des polymères de styrène; des produits de copolymérisation de l'oxyde d'éthylène avec un monomère hétérocyclique ou un monomère du type vinyle, des oligomères polyéther avec un poids moléculaire peu élevé; des particules de carbone; des zirconates trineoalkoxy amino; des zirconates trineoalkoxy sulfonyle; et des composés de la formule R-CH₂-N[CH₂CH₂O(C₂H₄O)_{y}(C₃H₆O)ₓZR']₂, où R est H ou C₁₋₉ alkyle, Z est un groupe difonctionnel modificateur de chaine, R' est H ou C₁₋₄ alkyle, et x et y sont entre 10 et 50.

8. Procédé selon la revendication 7, où R est H ou C₁₋₉ alkyle, R' est H ou C₁₋₄ alkyle et x et y sont entre 20 et 40.

9. Procédé selon la revendication 1, où l'agent antistatique comprend un polymère de l'oxyde d'éthylène et au moins un comonomère hétérocyclique.

10. Procédé selon la revendication 1, où l'agent antistatique comprend un mélange d'au moins un composé polaire organique avec au moins 5 atomes de carbone et un composé avec au moins 3 hétéroatomes.

11. Procédé selon la revendication 1, où l'agent antistatique comprend un acide sulfonique, un C₁₀-C-₁₆ alcane et des sels de sodium.

12. Procédé selon l'une quelconque des revendications précédentes, où l'agent antistatique comprend un ou plusieurs polyéthers, des éthers couronne, des polyoles, des polyimines, des polyamines, des polymères dérivés du pyridine, des composés azo macrocycliques, des polysulfides et des polyphosphines, et des sel d'acides protiques qui se trouvent solvatisés ou complexés dans un composé polaire organique.

13. Procédé selon l'une quelconque des revendications précédentes, où ledit niveau statique est entre -1 et 1 kilovolt par pouce (-51 et 51 kV/mm).

14. Procédé selon l'une quelconque des revendications précédentes, où au moins 5 % de la zone de surface de chaque filament est composée d'un polymère de nylon.

15. Procédé selon l'une quelconque des revendications précédentes, où au moins 5 % de la zone de surface totale de tous les filaments est composé d'un polymère de nylon.

16. Procédé selon l'une quelconque des revendications précédentes, comprenant les étapes: former un ou plusieurs mélanges fondus d'un polymère et d'un ou plusieurs agents antistatiques, soit dans un lot principal ou dans une résine basique, extruder dudit mélange ou des mélanges par des extrudeuses séparées en forme d'une pluralité de filaments à composantes multiples, où le mélange ou les mélanges d'un polymère et un ou plusieurs agents antistatique forment une zone de la surface des filaments, diriger les filaments é travers un dispositif d'atténuation, tirer les filaments pour les orienter, déposer les filaments sur une surface de collection pour former un tissu, et relier les filaments du tissu.

17. Procédé selon l'une quelconque des revendications précédentes, où l'étoffe est uniforme.
